

# UNITED STATES PATENT OFFICE.

CHARLES W. BULLOCK, OF BUFFALO, NEW YORK, ASSIGNOR, BY MESNE ASSIGNMENTS, TO FAIRSIMO GLUE COMPANY, INC., OF BUFFALO, NEW YORK, A CORPORATION OF NEW YORK.

## WATERPROOF GLUE OR CEMENT AND METHOD OF MAKING THE SAME.

1,124,286.

Specification of Letters Patent.

Patented Jan. 12, 1915.

No Drawing. Application filed March 24, 1911, Serial No. 616,576. Renewed May 22, 1914. Serial No. 840,363.

*To all whom it may concern:*

Be it known that I, CHARLES W. BULLOCK, a citizen of the United States, residing at Buffalo, in the county of Erie and State of New York, have invented a new and useful Improvement in Waterproof Glue or Cement and Method of Making the Same, of which the following is a specification.

This invention relates to a water and moisture-proof glue, cement or adhesive, and to the method of making the same.

The object of the invention is to produce a strong and thoroughly reliable and practical glue or cement suitable for gluing paper, wood, leather and various other substances, which is impervious to water and moisture, can be quickly and easily prepared for use, and is inexpensive to manufacture.

20 The glue or cement is composed of the following ingredients in approximately the proportions stated, to-wit: Animal glue, 90 ounces; zinc oxide, 8 ounces; chromic oxide, 8 ounces; lead carbonate, 16 ounces; and sufficient water to make 30 gallons of the solution, to which is added about 60 to 90 pounds of animal glue.

The product is made in the following manner: The first named amount (90 ounces) of glue is dissolved in 15 gallons (more or less) of water, after which the zinc oxide is added and the solution heated, preferably in a water bath, for about ten minutes. The chromic oxide and 5 gallons (more or less) of water are then added and the mixture is boiled for about 5 minutes. Then the lead carbonate and 10 gallons (more or less) of water are added and the mixture stirred thoroughly whereupon lead oxide is precipitated. After the precipitate has settled, the clear solution is preferably, though not necessarily, drawn off. Sixty to ninety pounds of glue is then added to the solution.

45 The above named proportions of the ingredients and the described method of making the glue can be varied somewhat and still produce a glue which is satisfactory for some purposes, but the described formula and method produce the most satisfactory glue or cement for general use.

The zinc oxide is used as a bleaching agent for the glue and to kill the animal fat therein. If glue is used which is free from fat and is sufficiently light in color; or if it contains zinc oxide, which is the case with some glue, then less zinc oxide is required, and it can even be omitted entirely in some cases.

55 Waterproof glue or cement made as above described is of a jelly-like consistency and 60 of whitish color. Before using the glue it is heated until it is thin enough to be readily spread in a thin even coat on the surfaces to be glued together. When the glue sets it forms a very strong adhesive, which is practically unaffected by water or moisture.

65 I claim as my invention:

1. A waterproof glue or cement comprising the following ingredients in approximately the proportions stated, to-wit:— 70 glue, 90 ounces; chromic oxide, 8 ounces; lead carbonate, 16 ounces; sufficient water to make a solution of 30 gallons, and additional glue, 60 to 90 pounds, substantially as set forth.

75 2. A waterproof glue or cement comprising the following ingredients in approximately the proportions stated, to-wit: glue, 90 ounces; zinc oxide, 8 ounces; chromic oxide, 8 ounces; lead carbonate, 16 ounces; 80 sufficient water to make a solution of 30 gallons, and additional glue, 60 to 90 pounds, substantially as set forth.

85 3. The herein described method of making waterproof glue or cement, consisting in dissolving 90 ounces (more or less) of glue in water; then adding 8 ounces (more or less) of zinc oxide and heating the solution; then adding 8 ounces (more or less) of chromic oxide and more water and boiling 90 the mixture; then adding 16 ounces (more or less) of lead carbonate and sufficient water to make about 30 gallons of the solution; and then adding 60 to 90 pounds (more or less) of glue, substantially as set 95 forth.

Witness my hand, this 15th day of March, 1911.

CHARLES W. BULLOCK.

Witnesses:

A. L. McGEE,  
C. W. PARKER.